

## UNITED STATES PATENT OFFICE

2,448,909

METHOD OF REMOVING INSULATION FROM  
METALLIC ELECTRIC CONDUCTORS

Yaro Piskac and Raymond E. Smiley, Maple Heights, Ohio, assignors, by means assignments, to Jack & Heints Precision Industries, Inc., Cleveland, Ohio, a corporation of Delaware

No Drawing. Application April 27, 1945,  
Serial No. 590,746

2 Claims. (CL. 134—38)

1

The present invention relates to the removal of insulating coatings from electrical conductors and the like and has for its primary object to provide a simple, effective and inexpensive process of chemically removing coatings of high dielectric strength and tough adhering characteristics as found in certain types of varnishes used for insulating purposes.

In practice it will be realized that it may be necessary to remove such insulation either locally to make electric connections or over a length of wire, or the like, when for example, the insulation has been damaged. The conventional practice has been to mechanically remove such insulation by scraping but this practice is laborious and time consuming and often results in irreparable damage to the conductor.

The present invention contemplates the convenient and expeditious removal of the insulation by a chemically active agent. There is a particularly effective insulation of high dielectric properties known in the trade as "Formvar," which is a vinyl acetate resin. It is a synthetic material, more-or-less in the nature of a plastic, and is used for coating electric conductors as an improvement over other known enamels used for insulating purposes. This material is extremely sticky and adhesive and difficult to apply. Such insulated conductors have found extensive use for the windings of generators, starter motors and the like and the "Formvar" insulation has been found to be extremely difficult to remove. It will be appreciated that the conventional procedure in applying such an insulation to a conductor is to apply it to the full length of the conductor. Subsequently, in order to make proper electrical connections, certain portions of the conductor must necessarily have its insulation removed. Besides removal of the varnish, dirt and organic material from the conductor the metallic surface should be removed and the surface of the conductor rendered clean and unimpaired and suitable for fusing as well as for electric current carrying purposes.

As a result of research and experimentation the present invention specifically contemplates for optimum results the use of an aqueous solution of a concentration of four pounds of chromium trioxide ( $\text{CrO}_3$ ) per gallon at a temperature of 221° Fahrenheit. The limit range of operation should preferably be kept within 10 to 14 grams of chromium trioxide per 25 cubic centimeters at

from 190° to 226° Fahrenheit. The optimum result under the preferred conditions above mentioned is the removal of insulation having characteristics comparable with that of "Formvar" within a period not exceeding 30 seconds.

Thus single wires or other conductors or a plurality thereof having "Formvar" insulation thereon may have any desired length adjacent their terminals, or in fact their entire length if desired, dipped into this solution at the preferred temperature and have the insulation quickly and thoroughly removed without damage to the conductor or its metallic surface.

We claim:

15. The method of removing insulation of vinyl acetate resin material from metallic electric conductors which comprises forming an aqueous solution of from ten to fourteen grams per 25 cubic centimeters of chromium trioxide, heating said solution to a temperature within a range of from 190° to 226° Fahrenheit and immersing a portion of said conductor with its insulation in said solution for a period of time approximating thirty seconds to remove said insulation without damage to said conductor or its metallic surface.
20. The method of removing insulation of vinyl acetate resin material from metallic electric conductors which comprises forming an aqueous solution of four pounds per gallon of chromium trioxide, heating said solution to a temperature of 221° Fahrenheit and immersing a portion of said conductor with its insulation in said solution for a period of time approximating thirty seconds to remove said insulation without damage to said conductor or its metallic surface.
25. The method of removing insulation of vinyl acetate resin material from metallic electric conductors which comprises forming an aqueous solution of four pounds per gallon of chromium trioxide, heating said solution to a temperature of 221° Fahrenheit and immersing a portion of said conductor with its insulation in said solution for a period of time approximating thirty seconds to remove said insulation without damage to said conductor or its metallic surface.

YARO PISKAC.  
RAYMOND E. SMILEY.

## REFERENCES CITED

The following references are of record in the file of this patent:

## UNITED STATES PATENTS

| Number    | Name         | Date          |
|-----------|--------------|---------------|
| 1,982,417 | Chandler     | Mar. 27, 1934 |
| 2,062,907 | Bessemberger | Sept. 1, 1936 |

## OTHER REFERENCES

50. Mellor "Modern Inorganic Chemistry," Longmans, Green and Co., N. Y., 1939 (page 772 relied on). (Copy in Division 27.)